

Patented Apr. 24, 1945

2,374,565

# UNITED STATES PATENT OFFICE

2,374,565

## RUST PREVENTIVE COMPOSITIONS

Harry Roden, Port Neches, Tex., assignor, by  
mesne assignments, to The Texas Company,  
New York, N. Y., a corporation of Delaware

No Drawing. Application May 31, 1941,  
Serial No. 396,169

6 Claims. (Cl. 106—14)

This invention relates to a non-drying rust preventive composition adapted for use on unclean corroded surfaces, and particularly such metallic surfaces as are exposed to severe corrosive conditions resulting from acids and salt brine. These compositions are designed to react upon the corroded metallic surface in such a manner as to separate the chemically-laden rust from the base metal and provide a protective film on the base metal which repels any corrosive action of the surrounding media and prevents further encrustation of the existing chemical rust. In order for such compositions to be effective they must be able to penetrate through a body of rust and surround and isolate the rust particles so that the particles are rendered inactive and free from the base metal. Further, these compositions must possess the property of "self-healing" which may be interpreted as the flowing or leveling off of the protective film to "heal" any scratches or abrasions occurring after application, or such rough or pitted areas which may be "bridged over" during the application so that the resulting protective film covers the entire area of the base metal to be protected. As distinguished from the former drying films, these compositions should be moisture-proof and should not soften or hydrolyze under continued water submersion, with the resultant effect that any undermining, due to the pressure of moisture, is reduced to a minimum.

The present invention is based upon the discovery of a class of grease-type non-drying rust preventive compositions which possess all the above-mentioned properties. These compositions are composed of a homogeneous mixture of mineral oil, amorphous mineral oil wax, wool fat material, and esters and/or salts of high molecular weight carboxylic acids. Since the requirements of these compositions are so stringent and their service conditions so severe in that they are exposed to all types of corrosive conditions, such properties as melting point, penetrating ability, wetting power, texture and hardness, become prime factors. It has been ascertained that these properties are directly affected by the type and quantity of the individual components of composition and their relation one to the other, as, for example, the wax content, the kind of mineral oil used, the ratio of wool fat to wax, the quantity and viscosity of the oil, the proportions of esters used, etc. Taking into consideration all these factors, it has been found that the optimum proportionate range of the individual components lie between the following limits:

|                                                               | Per cent |
|---------------------------------------------------------------|----------|
| Amorphous mineral oil wax                                     | 50-85    |
| Mineral oil                                                   | 15-40    |
| Wool fat                                                      | 1-8      |
| Esters and/or salts of high molecular weight carboxylic acids | 0.4-6    |

These components may further consist of mix-

tures of constituents falling within the general types, mentioned and may be varied within the above-mentioned limits to accentuate the particular properties desired. Thus, the amorphous mineral oil wax content which includes petrolatum in its classification, may be divided into two or more constituents of varying melting points. In the preferred form, the amorphous mineral oil wax, which constitutes 50-85% of the composition, is divided into a mixture of a high and low melting point petrolatum in the following proportionate range:

|                                | Per cent |
|--------------------------------|----------|
| Petrolatum (140-150° F. M. P.) | 50-70    |
| Petrolatum (150-165° F. M. P.) | 0-15     |

The mineral oil component is effective in preventing hardening of the composition and aids in giving the desired texture and penetrating ability. It has been found desirable to provide a blend of mineral oils of varying bases and viscosity ranges, such as approximately two parts of a residual oil to one part light oil distillate. Among the various oils which may be blended to impart the desired structure and hardness to the final composition are the various base and viscosity cylinder stocks and pale oils. The preferred blends of the mineral oils, as present in the final composition, consist of 10-25% of a cylinder stock within the Saybolt Universal viscosity range of 115-215 at 210° F., and 5-15% of a viscous pale oil within the Saybolt Universal viscosity range of 150-250 at 100° F.

The wool fat material is used as a flux and adhesive and possesses excellent wetting powers at low temperatures. This material may be either degras or the esters and acids of wool fat. The final component, namely the esters and/or salts of high molecular weight carboxylic acids, have been found to possess exceptional wetting, penetrating, texture improving, and cohesive properties when present in compositions of this type in proportions of from 0.4 to 6%. Among the esters and salts found to be particularly suitable are the heavy metal salts and alkyl esters of fatty acids, and particularly the high molecular weight fatty acids of the type of stearic acid. The alkyl radical of the alkyl esters preferably contain from 1-5 carbon atoms. These esters and salts may be used singly or in combination with one another, depending upon the type of properties desired in the final composition. However, when using a combination of these two, it is preferred to have them present in the final product within the following proportionate ranges:

|                  | Per cent |
|------------------|----------|
| Heavy metal salt | 0.4-1.0  |
| Alkyl ester      | 1-5      |

In preparing the composition, the cylinder stock is first added to a kettle at room temperature and the heavy metal salt of a fatty acid added thereto. The mixture is then stirred without heating until the mass is uniform, at which

